

## UNITED STATES PATENT OFFICE

2,328,198

LOW ELECTRICAL RESISTANCE PAPER AND  
METHOD OF MAKING SAMEFranklyn E. Davenport, David C. Knowlton, and  
Robert W. McCormick, Watertown, N. Y., as-  
signors to Knowlton Bros., a corporation of  
New YorkNo Drawing. Application April 12, 1939,  
Serial No. 267,468

18 Claims. (Cl. 92—21)

This invention relates to fibrous materials such as paper or the like having an extremely low electrical resistance to be very highly conductive to electricity rather than being dielectric or an insulator thereof, and more particularly pertains to the use of fibrous material of this character, when provided with suitable coating sensitive to the passage of electricity, in an apparatus for having reproduced thereon in facsimile marks, characters, designs, pictures or the like which are transmitted by wire or radio.

Finely divided mineral and inert materials and the like have heretofore been used in the manufacture of paper, these materials being used as a filler incorporated in the pulped mass from which the paper is formed or applied as a coating to one or both surfaces of the sheet fabricated from the pulped mass. Or the filling material is incorporated in the pulped mass, and the fabricated filler containing sheet may also be coated with the mineral or inert material containing compound. In whatever way the filling materials have been associated with the sheet, their purpose has been to fill the interstitial spaces within the body of the sheet or those spaces on its surfaces and/or to give color to the sheet. The filling materials give closer texture to the sheet, enable it to be more highly finished and color same. Kaolin, talc, clay and the like are the chief filler substances used for loading the paper. Paper made of fiber alone is more or less translucent, the degree of translucency depending on its thickness and on the nature of the fibrous material. Some kinds of fiber are more dense and opaque than others. The filling material overcomes translucency and gives opaqueness and color together with the other mentioned advantages.

It is the aim of the present invention to employ filling material or materials which are very highly conductive to electricity and to disperse same thoroughly through the body of the fibrous sheet so that said filler containing or loaded fibrous sheet is also very highly conductive to electricity, thereby making said sheet useful where highly conductive sheets are employed and particularly adapted as a base to which a coating may be applied to make the paper suitable for use in an apparatus on which facsimile messages or the like are to be reproduced.

Generally described, the finely divided materials of highly conductive character are intimately dispersed in water to form what may be called a colloidal solution. Carbonaceous and

graphitic materials, metals and the like are representative of suitably highly conductive fillers. Paris black, gas-carbon and graphite are representative of carbonaceous and graphitic materials. Aluminum powder is representative of a suitable metallic material. All of the finely divided materials are electric conductive materials of the first class. The colloidal solution is then incorporated in a beater with a batch of fibrous stock, and beaten to a suitable freeness which is adapted to be fabricated in a loosely or compactly felted sheet on any conventional paper-making apparatus. Other components, such as size and papermakers' alum may be incorporated in the batch if desired. The felted sheet is supercalendered and may be machine calendered before being supercalendered.

A sheet thus constructed is then treated on one or both sides with any suitable coating sensitive to an electric current and employed for coating sheets which are to be printed by a stylus or styl through which electrical impulses are transmitted for reproducing messages and the like on the sheet. That is, the coating has the property of changing color at selected areas where electric current is passed through, thereby contrasting these areas in color with the remaining areas of the coating through which the electric current is not passed and causing letters, characters and the like to be formed. The coating is usually white in color. The sheets are particularly adapted for use on what is known as the Finch machine, and other machines which print by electrical impulses on sheets sensitive to electricity. Facsimile recorders of the former are shown in Finch Patents 2,141,974 and 2,141,975 issued December 27, 1938. These are representative of machines having a stylus mounted on an arm which is adapted to oscillate over the paper to receive the facsimile printing.

The invention is more specifically described by giving one preferred formula which has been found satisfactory in commercial use. This formula comprises about one thousand pounds (1000 lbs.) of fibrous material, such as rags, wood pulp or the like, and about one hundred and fifty pounds (150 lbs.) of Paris black, otherwise known as lamp black or carbon black. These are not critical proportions and they may be varied within a wide range. Any finely divided granular material having a high carbon content appears to be particularly suitable.

The Paris black is preferably very finely divided so that same may be thoroughly dispersed in water. To thoroughly disperse the Paris black

in the water, the mixture is agitated. Dispersion may be accelerated by heating the mixture before or during agitation. Any mixer or agitator may be used which can be manipulated to thoroughly disperse the Paris black in water. While there is no limitation as to the time of mixing and agitating or the manner of mixing, it has been found that with a high speed motor-driven mixer the Paris black can be sufficiently dispersed in the water in about fifteen minutes. About fifty gallons (50 gals.) of water may be used advantageously for about thirty-seven and one-half pounds (37½ lbs.) of Paris black. These proportions are not critical but merely illustrative and may vary with a considerable wide range.

The Paris black and water mixture or colloidal solution is then mixed with the fibrous pulp material which is then processed in any conventional beater commonly employed in the paper industry for beating fibrous stock. The fibrous stock, if desired, may be beaten wholly or partially before the Paris black and water mixture is incorporated therein.

It is important that the Paris black be thoroughly and intimately mixed in and throughout the pulped mass, and to obtain a sufficient intermixture the Paris black is preferably first dispersed in water before being associated with the fibrous material, as more thorough distribution of the finely divided material throughout the furnish stock is obtained. The Paris black is very finely divided and of the character of fine powder or dust.

A size may be added to make the paper less absorbent or porous, to give a good surface and impart the proper degree of stiffness. It fills up the pores between the fibers and gives a finer texture. If a size is used, rosin is preferable and may be added best in the beater.

A small quantity of papermaker's alum or aluminum sulphate is preferably used, particularly if a size is added to the furnish stock. The dry alum can be put in the beater, but a solution with water is better. The function of the alum is to fix the filler material.

The pulped mass of the composition above described and beaten to the proper consistency is run into a stock chest or a number of them or to a Jordan or other refining engine if further refining of the furnish stock is desired.

The refined stock is then felted on a conventional paper-making machine of the cylinder or Fourdrinier type and calendered, the calender compressing and ironing the sheet to provide a smooth finish. However, the conventional machine calendering alone, which comprises passing the formed sheet from the paper-making machine between a series of vertically disposed steel rolls, is not alone sufficient to give the very high conductivity characteristic to the sheet. The machine calendered sheet is then immediately or subsequently, after being seasoned, passed through a supercalender. A conventional supercalender has a number of polished rolls for giving a higher compression and more finish to the paper than can be obtained by the machine calenders. While the sheet is more highly finished by reason of the supercalendering, it appears that the higher pressure to which the sheet is subjected in the supercalender operation brings the finely divided and thoroughly distributed conductive particles into closer association if not into actual contact, thereby providing a substantially continuous medium for conducting electric current through the body or thickness of the paper.

This higher pressure of the paper beyond the mill or machine compression obtained by the conventional machine calender may for convenient reference be designated "super-compressed" and the finish resulting from same as "super excellent." Without the pressure exerted by supercalendering, the distributed finely divided and thoroughly distributed particles are more separated from each other by the fibers. Possibly there may be other factors causing or contributing to the qualities and characteristics obtained in the sheet, and thus this view is advanced as a theory rather than a fact. There is the fact that a mechanical operation, such as supercalendering, gives a paper of the composition above described, its quality of high conductivity to electricity whatever may be the reason for it.

Supercalenders usually comprise seven to eleven rolls, more or less, in a stack, part of the rolls being chilled polished metal and part being cotton or paper rolls. The metal and cotton or paper rolls may or may not be alternately disposed.

The supercalendered sheet is manufactured and sold as an article of manufacture, and while it may have other uses it is especially suitable as a base sheet which is to be coated on one or both sides with any suitable coating which is sensitive to electricity, thereby being adapted to have electrically reproduced thereon messages and the like which are transmitted by wire or radio. The invention is not limited to any particular coating material. Any which is adapted to be changed in color by an electric current is suitable.

The base sheet is very thin, preferably from three to four thousandths (.003 to .004) of an inch. The electrical resistance of a paper thus fabricated when measured on a Wheatstone bridge at six volts between contacts of weight of about 300 grams and an area of about 3.546 square inches is less than one thousand (1000) ohms, although the invention is not thus limited. The area is that of a circle resulting from a diameter of about 2½ inches. A suitable sheet may be as high or higher than ten thousand (10,000) ohms.

Paris black is jet black in color, and the fabricated sheet, if Paris black is used as the filling material, is black. While Paris black is preferable, other filling materials of the same general character, except as to color, would be suitable. Finely divided metals are suitable but are, of course, more expensive than Paris black. Finely divided material having a high carbon content is especially suitable. The finely divided materials which are suitable are those highly conductive to electricity. Thus, suitable filling materials are determined by their quality of being highly conductive to electricity rather than as to kind. They should also be capable of ready dispersion in water.

While one particular formula has been described in detail for carrying out the invention, and a particular use for the sheet has been referred to, it will be understood that there may be changes in details of composition and manufacture without departing from the spirit of the invention, and that the sheet may have other uses where a sheet having a high conductivity quality is desired.

Having described our invention, we claim:

1. A paper of low resistance to electricity formed from a furnish stock composed of refined fibrous material and finely divided electrical conductive material of the first class intimately commingled in proportions, by weight, of approxi-

mately six and two-thirds times as much refined fibrous material as conductive material and compressed more highly and given more finish than obtained by a machine calender to render said paper highly conductive to electricity.

2. A paper of low resistance to electricity formed from a furnish stock composed of refined fibrous material and finely divided carbonaceous material intimately commingled in proportions, by weight, of approximately six and two-thirds times as much refined fibrous material as conductive material and compressed more highly and given more finish than obtained by a machine calender to render said paper highly conductive to electricity.

3. A paper of low resistance to electricity formed from a furnish stock composed of refined fibrous material and finely divided material of a high carbon content intimately commingled in proportions, by weight, of approximately six and two-thirds times as much refined fibrous material as conductive material and compressed more highly and given more finish than obtained by a machine calender to render said paper highly conductive to electricity.

4. A paper of low resistance to electricity formed from a furnish stock composed of refined fibrous material and finely divided electrical conductive material of the first class intimately commingled and supercalendered to render said paper highly conductive to electricity.

5. A facsimile recording paper through which electricity is adapted to be passed and which is of low resistance to electricity formed from a furnish stock composed of refined fibrous material and finely divided electrical conductive material of the first class intimately commingled in proportions, by weight, of approximately six and two-thirds times as much refined fibrous material as conductive material and compressed more highly and given more finish than obtained by a machine calender to render said paper highly conductive to electricity, and a coating on the paper which is sensitive to electric current for being changed in color when electricity is passed through the paper.

6. A facsimile recording paper through which electricity is adapted to be passed and which is of low resistance to electricity formed from a furnish stock composed of refined fibrous material and finely divided carbonaceous material intimately commingled in proportions, by weight, of approximately six and two-thirds times as much refined fibrous material as conductive material and compressed more highly and given more finish than obtained by a machine calender to render said paper highly conductive to electricity, and a coating on the paper which is sensitive to electric current for being changed in color when electricity is passed through the paper.

7. A facsimile recording paper through which electricity is adapted to be passed and which is of low resistance to electricity formed from a furnish stock composed of refined fibrous material and finely divided material of a high carbon content intimately commingled in proportions, by weight, of approximately six and two-thirds times as much refined fibrous material as conductive material and compressed more highly and given more finish than obtained by a machine calender to render said paper highly conductive to electricity, and a coating on the paper which is sensitive to electric current for being changed

in color when electricity is passed through the paper.

8. A facsimile recording paper through which electricity is adapted to be passed and which is of low resistance to electricity formed from a furnish stock composed of refined fibrous material and finely divided electrical conductive material of the first class intimately commingled and supercalendered to render said paper highly conductive to electricity, and a coating on the paper which is sensitive to electric current for being changed in color when electricity is passed through the paper.

9. A paper of low resistance to electricity formed in thickness from about three to four thousandths of an inch from a furnish stock comprising about one thousand (1000) pounds of refined fibrous material and about one hundred and fifty (150) pounds of Paris black intimately commingled and supercalendered to provide an electrical resistance not substantially exceeding ten thousand (10,000) ohms measured over the area of a circle resulting from a diameter of about two and one-eighth (2 1/8) inches.

10. A facsimile recording paper through which electricity is adapted to be passed and which is of low resistance to electricity formed in thickness from about three to four thousandths of an inch from a furnish stock comprising about one thousand (1000) pounds of refined fibrous material and about one hundred and fifty (150) pounds of Paris black intimately commingled and supercalendered to provide an electrical resistance not substantially exceeding ten thousand (10,000) ohms measured over the area of a circle resulting from a diameter of about two and one-eighth (2 1/8) inches, and a coating on the paper which is sensitive to electric current for being changed in color when electricity is passed through the paper.

11. A method of fabricating a paper of low resistance to electricity comprising forming a colloidal solution of water and finely divided electrically conductive material of the first class, intimately commingling the solution with a furnish stock of fibrous pulp, felting the furnish stock into a sheet, calendering and supercalendering the felted sheet.

12. A method of fabricating a paper of low resistance to electricity comprising forming a colloidal solution of water and finely divided material having a high carbon content, intimately commingling the solution with a furnish stock of fibrous pulp, felting the furnish stock into a sheet, calendering and supercalendering the felted sheet.

13. A method of fabricating a facsimile recording paper through which electricity is adapted to be passed and which is of low resistance to electricity comprising forming a colloidal solution of water and finely divided electrically conductive material of the first class, intimately commingling the solution with a furnish stock of fibrous pulp, felting the furnish stock into a sheet, calendering and supercalendering the felted sheet, and coating the supercalendered sheet with a coating which is sensitive to electric current for being changed in color when electricity is passed through the sheet.

14. A method of fabricating a facsimile recording paper through which electricity is adapted to be passed and which is of low resistance to electricity comprising forming a colloidal solution of water and finely divided material having a high carbon content, intimately commingling the solu-

tion with a furnish stock of fibrous pulp, felting the furnish stock into a sheet, calendering and supercalendering the felted sheet, and coating the supercalendered sheet with a coating which is sensitive to electric current for being changed in color when electricity is passed through the sheet.

15. A method of fabricating a paper of low resistance to electricity comprising rapidly agitating finely divided particles of electricity conducting material of the first class with water to intimately commingle same, mixing the aqueous mixture with a refined furnish stock of fibrous material, felting a sheet from the furnish stock, calendering and supercalendering the sheet to compress same and bring the conductive particles in close association.

16. A method of fabricating a paper of low resistance to electricity comprising rapidly agitating finely divided particles of electricity conducting material of the first class with water, in proportions of about thirty-seven (37) pounds of the finely divided material to fifty (50) gallons of water, to intimately commingle same, mixing the aqueous mixture with a refined furnish stock

of fibrous material, felting a sheet from the furnish stock, calendering and supercalendering the sheet to compress same and bring the conductive particles in close association.

5 17. A paper of low resistance to electricity formed from a furnish stock composed of refined fibrous material and an aqueous colloidal solution of finely divided electrical conductive material of the first class intimately commingled and supercalendered to render said paper highly conductive to electricity.

10 18. A paper of low resistance to electricity formed from a furnish stock composed of refined fibrous material and an aqueous colloidal solution of finely divided electrical conductive material of the first class intimately commingled and supercalendered to render said paper highly conductive to electricity, and a coating on the paper which is sensitive to electrical current for being changed in color when electricity is passed through the paper.

25

ROBERT W. McCORMICK.  
DAVID C. KNOWLTON.  
FRANKLYN E. DAVENPORT.